

# United States Patent

Boyer

[15] 3,658,603  
[45] Apr. 25, 1972

[54] SURFACE FINISHING

[72] Inventor: Charles D. Boyer, Natrona Heights, Pa.  
[73] Assignee: Allegheny Ludlum Steel Corporation, Pittsburgh, Pa.  
[22] Filed: Jan. 2, 1970  
[21] Appl. No.: 437  
  
[52] U.S. Cl.....148/6.16, 117/127, 148/6.27  
[51] Int. Cl.....C23f 7/10, C23f 7/13  
[58] Field of Search.....148/6.16, 6.15 Z, 6.35, 6.27;  
117/169, 127

[56] References Cited

UNITED STATES PATENTS

2,753,282 7/1956 Perry .....148/6.16  
3,125,471 3/1964 Conner .....148/6.35 X  
1,947,122 2/1934 Burdick et al. .....148/6.16  
3,248,250 4/1966 Collins.....148/6.16 X

3,248,251 4/1966 Allen .....148/6.16 X

Primary Examiner—Ralph S. Kendall  
Attorney—Richard A. Speer, Vincent G. Gioia and Howard R. Berkenstock, Jr.

[57]

## ABSTRACT

A method of providing a decorative exposed metallic surface with protection from marring, marking and staining, comprising the steps of coating the surface with an aqueous solution which contains ions of magnesium, ammonium, chromate and phosphate and curing said coating.

A composite article comprising a layer of metal having a decorative exposed surface and at least one layer of a substantially water insoluble, transparent, cured coating which offers protection from marring, marking and staining. The cured coating being comprised of magnesium cations and anionic polymeric chains of chromium, oxygen and phosphorus atoms.

24 Claims, No Drawings

## SURFACE FINISHING

The present invention relates to a method for protecting a decorative metallic surface from marring, marking and staining and to a composite article comprising a layer of metal and a coating which protects the metal from marring, marking and staining.

Numerous articles of manufacture, such as water fountains and building panels, have decorative metallic surfaces; e.g., stainless steel. These surfaces are in need of protection as they are subjected to severe abuse. They are scratched, smeared by natural skin oils and other contaminants found on hands, weathered by various atmospheric conditions and stained by different solvents and chemicals.

Considerable time and money has been spent on developing coatings which will protect metallic surfaces. I have discovered that cured coatings of magnesium cations and anionic polymeric chains of chromium, oxygen and phosphorus atoms protect metal surfaces without detracting from their appearance.

It is accordingly an object of this invention to provide a method for protecting a decorative metallic surface from marring, marking and staining.

It is another object of this invention to provide a composite article comprising a layer of metal and a coating which protects the metal from marring, marking and staining.

The method of this invention comprises the steps of coating the metal to be protected with an aqueous solution which contains ions of magnesium, ammonium, chromate and phosphate and curing the coating so as to render it substantially water insoluble. In this application, the term phosphate ion includes all ions related to phosphoric acid in an aqueous solution. Thus, the species  $H_3PO_4$ ,  $H_2PO_4$ ,  $HPO_4$  and  $PO_4$  and any polymeric phosphorous oxyacid anions are collectively referred to as phosphate ion. Similarly,  $CrO_3$  in solution may exist as  $CrO_4$ ,  $Cr_2O_7$ , etc., as well as in various protonated forms, all of which are included in the term chromate ion.

The ions; i.e., magnesium, ammonium, chromate and phosphate, may be supplied in various ways. Magnesium ion may be supplied as the oxide, hydroxide, carbonate, bicarbonate, phosphate or chromate. Ammonium ion may be supplied as uncombined ammonia, aqueous ammonium hydroxide, or as the phosphate, chromate, carbonate or bicarbonate salts. Phosphate ion is most conveniently supplied as orthophosphoric acid. It can also be supplied as magnesium phosphate, ammonium phosphate or magnesium ammonium phosphate. Chromate ion may be supplied as chromium trioxide or as the chromate or dichromate salts of magnesium or ammonium. When the ammonium or magnesium ions are supplied as their phosphate or chromate salts, the composition ratios of the solution are limited to the composition ratios of the particular salts used. Variations of these composition ratios can, however, be produced by adding extra magnesium or ammonium as one of the other acceptable compounds. The most convenient method for producing the coating solution is to use magnesium hydroxide, ortho-phosphoric acid, concentrated aqueous ammonium hydroxide and chromium trioxide.

The magnesium, ammonium, chromate and phosphate ions are proportionately present in the aqueous solution as 0.01 - 28 mole percent magnesium ion, 5 - 22 mole percent ammonium ion, 4 - 26 mole percent chromate ion and 33 - 67 mole percent phosphate ion and preferably as 16 - 26 mole percent magnesium ion, 7 - 15 mole percent ammonium ion, 7 - 21 mole percent chromate ion and 45 - 65 mole percent phosphate ion. Magnesium is needed in order to render the cured coating substantially water insoluble and to decrease curing times to reasonable periods. A lower limit of 0.01 mole percent magnesium ion is imposed as cured coatings formed from solutions with less than 0.01 mole percent are not water insoluble. An upper limit of 28 mole percent magnesium ion is imposed as 28 mole percent is the limit of the solubility for magnesium ion in the coating solution. Chromate ion assists in giving the coating its transparency and is required to render the coating substantially water insoluble after curing. Solutions with less than 4 percent chromate ion produce opaque

cured coatings and solutions with more than 26 mole percent chromate ion produce blotchy coatings which require excessive curing times. Ammonium ion also assists in giving the coating its transparency. Solutions with less than 5 and more than 22 mole percent ammonium ion produce opaque cured coatings. Phosphate ion is required to render the solution acidic. A minimum phosphate ion level of 33 mole percent is necessary in order for the other ions of the solution to adequately dissolve. An upper limit of 67 mole percent phosphate ion is set, as good curing and clarity will not be obtained at higher levels. When the phosphate ion is in excess of 67 mole percent, there is a deficiency of other ions.

The concentration of magnesium, ammonium, chromate and phosphate ions in the water should be no greater than about 1.5 moles of ions per 100 ml. of water and preferably should be no greater than 0.8 moles of ions per 100 ml. of water. Solutions with concentrations in excess of 1.5 have too high a solid level and produce a cloudy, bubbly coat. On the other hand, there does not appear to be a minimum concentration of ions in the water.

Any composition which gives a transparent coating will continue to give a transparent coating as the amount of water is increased. The only effect of dilution is to decrease the coating thickness. For practical purposes a lower limit of 0.01 moles of ions per 100 ml. of water has been set. A preferred lower limit is 0.25 moles of ions per 100 ml. of water.

A wetting agent can be added to the coating solution to insure the best possible wetting action at the metal surface. The use of wetting agents is optional and by no means necessary.

Typical wetting agents are Wetanol (Glyco Products, Inc., New York, N.Y.) and Alkanol HCS (E. I. du Pont de Nemours & Company, Wilmington, Del.). Any of the well-known coating methods can be employed.

The invention is not dependent upon the use of any particular coating method. Illustrative coating methods are dip coating, flow coating, spray coating, roll coating and spin coating.

The coating should be cured so as to render it substantially water insoluble. Curing is a time and temperature dependent process.

Shorter times are required at higher temperatures and longer times are required at lower temperatures. Curing temperatures; i.e., the temperatures at the metallic surfaces, ranging from 400° to 1,900° F. have been successfully employed at times ranging from two seconds to four hours.

Various colors and tints can be given to the coating by varying the curing temperature. This enables certain metals; e.g., stainless steel, to take on the appearance of color without treating; e.g., heat tinting, the metal. Color can also be varied by adjusting the relative proportion of magnesium, ammonium, chromate and phosphate ions which are present in the aqueous coating solution and/or by adjusting the thickness of the cured coating. It is also within the scope of this invention to add pigments, dyes and other chemical agents to alter the color of the coating.

The article of this invention is comprised of a layer of metal having a decorative surface disposed to be visible and at least one layer of a substantially water insoluble, transparent, cured coating which offers protection from marring, marking and staining, disposed in adhering relation on the decorative surface. The coating is comprised of magnesium cations and anionic polymeric chains of chromium, oxygen and phosphorous atoms. No limit is placed on the thickness of the coating although each individual layer should not exceed 0.0005 inches. Layers thicker than 0.0005 inches require an excessive amount of coating solution and acquire a frosty appearance during curing.

Although the invention is believed to be adaptable to a wide variety of metallic surfaces which include stainless steel, brass, aluminum, silver, zinc, copper, plain carbon steel, lead, chromium, nickel, gold plate, black chrome and platinum; stainless steel is probably the most important decorative metal and, accordingly, the following is directed to stainless steel embodiments. Stainless steel has a strikingly noticeable tendency to show scratches and marks which cannot be easily

removed by any known commercial means without destroying its uniform appearance.

Stainless steel trim members; e.g., automotive trim members, having a contact surface which abuts a metallic body member less noble in the electromotive series than stainless steel; e.g., a carbon steel automotive body, and an exposure surface subject to view, constitute a particular embodiment of this invention. Another particular embodiment are assemblies comprised of stainless steel trim members and metallic body members.

Stainless steel is known to serve a particularly good purpose in those applications where brightness and corrosion resistance is required and is ideally suited for use as automotive trim. However, since most automotive bodies are constructed of carbon steel, the use of stainless steel can result in galvanic corrosion. Carbon steel is anodic to stainless steel and generally corrodes in the vicinity of stainless steel in the presence of an electrolyte, such as moisture. Galvanic corrosion can, however, be precluded if an insulating material is placed between the carbon steel and the stainless steel; e.g., on the contact surface of the stainless steel trim member. The coating described in this application is particularly appropriate since it will serve as an insulator and will also provide the exposure surface with protection from marring, marking and staining.

The following examples illustrate several aspects of the invention.

#### EXAMPLE I

A.I.S.I. Type 434 stainless steel samples 0.0185 inches thick were dip coated in an aqueous solution containing ions of magnesium, ammonium, chromate and phosphate. The ions were proportionately present in the solution as 22.5 mole percent magnesium ion, 9.5 mole percent ammonium ion, 12.5 mole percent chromate ion and 55.5 mole percent phosphate ion. The molar concentration of the specified ions in the solution was 0.420 moles of ions per 100 ml. of water. Half of the samples had a bright anneal finish and half had a matte finish. All the samples were cured for one minute in a furnace at temperatures ranging from 550° F. up to 1,200° F. The bright annealed samples had coatings ranging from 0.000040 inches to 0.000168 inches and the matte finished samples had coatings ranging from 0.000043 inches to 0.000209 inches. Table I, found below, gives the appearance of the coating. Note how the appearance changes with the curing temperature.

TABLE I

| Curing Time (Mins.) | Curing Temperature (°F.) | Appearance On Type 434 B.A. Finish | Appearance On Type 434 Matte Finish |
|---------------------|--------------------------|------------------------------------|-------------------------------------|
| 1 min.              | 550                      | Dark Gold                          | Medium Yellow Gold                  |
| "                   | 600                      | Medium Gold                        | Brownish Gold                       |
| "                   | 700                      | Light Yellow Gold                  | Tannish Gray                        |
| "                   | 800                      | Yellow Gold Tint                   | Light Gray, Tan Tint                |
| "                   | 850                      | Tan Tint                           | Light Gray, Tan Tint                |
| "                   | 900                      | Substantially Colorless            | Gray-Green                          |
| "                   | 950                      | Substantially Colorless            | Tint                                |
| "                   | 1000                     | Substantially Colorless            | Gray-Green                          |
| "                   | 1100                     | Light Cloudy Gray                  | Tint                                |
| "                   | 1200                     | Cloudy Blue Gray                   | Gray, Gray-Tan                      |

The bright annealed and the matte finished samples which were cured at 900° F. and 1,000° F. were subjected to a number of tests. The favorable results of the tests are reported below.

70  
75

#### SOLVENT, ACID AND ALKALI RESISTANCE

No deterioration of the coating was revealed after the samples were immersed in acetone, methyl acetate, benzene, kerosene, methyl ethyl ketone, toluene, methyl alcohol and xylene for a 5-day period.

Concentrated and dilute solutions of nitric, hydrochloric, phosphoric, and acetic acids did not damage the coating after 24 hours of exposure.

10 Concentrated and dilute hydrofluoric acid caused some deterioration of the coating. Concentrated hydrofluoric discolored the coating after 4 hours. Dilute hydrofluoric caused a stain at the interface of the coating and metallic surface after 6 hours.

15 Concentrated and dilute concentrations of sulfuric acid caused some slight pitting of the sample under the coating. The continuity; e.g., electrical resistance, of the coating was not, however, affected after 24 hours of testing.

Concentrated and dilute ammonium hydroxide did not affect the coating after 6 hours.

20 Sodium hydroxide at concentrations of 61 percent and 10 percent did not affect the coating after 6 hours. A 25 percent concentration of sodium hydroxide heated to a temperature of 200° F., removed all the coating in 5 to 10 minutes.

#### SOIL AND ABRASION RESISTANCE

Fingermarks and various types of soil were placed on the coating and easily removed by wiping.

30 A bright annealed sample was tested with an abrasion tester. Two one-half inch wide  $\times$  2½ inch diameter rubberized boron wheels, each causing a 1,000 gram drag on the coated surface, traveled over a 3½ inch diameter circle while being driven by the samples which were revolved. Any coating that will withstand 100 cycles of this test is considered to be very good. The tested coating withstood 800 cycles without having its continuity impaired. This indicates that it is very hard and should offer high resistance to marking and marring.

#### ATMOSPHERIC ENVIRONMENT RESISTANCE

Coated samples which were placed in a humidity cabinet, where the humidity was controlled at 92 percent, revealed no efflorescence or any other detrimental effect.

Coated and uncoated samples were placed on cars in the Pittsburgh, Pa., area for evaluation in a "Winter Corrosion Program" — galvanic corrosion was evident on the cars which had the uncoated samples, but was not evident on the cars which had the coated samples.

50 A bright annealed sample was tested in a Weather-Ometer for 2,292 hours with no apparent damage to the coating. This is considered to be the equivalent of seven years of atmospheric exposure.

#### FORMABILITY RESISTANCE

No adverse results were observable on sheared samples. Crazing was observable on the convex side of a coated sample after bending.

#### EXAMPLE II

Two A.I.S.I. Type 304 stainless steel strips 0.025 inches thick were roll coated with two different aqueous solutions containing ions of magnesium, ammonium, chromate and phosphate. One of the strips had a bright anneal finish and the other had a brushed finish. Table II, found below, gives the general concentration in which the ions were proportionately present in the solutions.

TABLE II

| Ions          | Solution A (Mole %) | Solution B (Mole %) |
|---------------|---------------------|---------------------|
| Magnesium Ion | 22.8                | 21.3                |
| Chromate Ion  | 12.4                | 18.4                |

|               |      |      |
|---------------|------|------|
| Phosphate ion | 55.1 | 51.5 |
| Ammonium ion  | 9.5  | 8.8  |

The molar concentration of the ions in solutions A and B were respectively 0.91 and 1.05 moles of the specified ions per 100 ml. of water.

The coated strips were divided into a number of samples which were cured at temperatures ranging from 630° to 1,030° F. for a period of 2 minutes. The samples were subsequently measured for color. Color values were obtained using a Hunter Associates (Mclean, Va.), Laboratory Sphere Color and Color - Difference Meter, Model D25.

Table III, found below, gives the finish of the samples prior to coating, the coating solution used, the curing temperature, the calculated coating thickness after curing and the color values.

TABLE III

| Sample | Finish        | Coating solution | Curing temp. (°F) | Thickness of coating (micro inches) | Color |      |       |      |      |
|--------|---------------|------------------|-------------------|-------------------------------------|-------|------|-------|------|------|
|        |               |                  |                   |                                     | L     | a    | b     | ΔE   | Haze |
| 1.     | Brushed       | Uncoated         |                   |                                     | 65.5  | -0.5 | +2.6  | 0    | 88.5 |
| 2.     | do            | A                | 630               | 42                                  | 62.9  | -0.8 | +8.4  | 6.3  | 79.2 |
| 3.     | do            | A                | 730               | 52                                  | 63.1  | -1.5 | +7.8  | 5.8  | 78.8 |
| 4.     | do            | A                | 830               | 73                                  | 63.0  | -1.5 | +6.1  | 4.5  | 80.2 |
| 5.     | do            | A                | 930               | 58                                  | 62.2  | -1.3 | +5.4  | 4.4  | 79.7 |
| 6.     | do            | A                | 1030              | 71                                  | 62.2  | -1.3 | +4.5  | 3.9  | 80.2 |
| 7.     | do            | B                | 630               | 60                                  | 56.8  | +0.8 | +17.7 | 17.5 | 77.5 |
| 8.     | do            | B                | 730               | 51                                  | 59.4  | -0.4 | +11.3 | 10.6 | 84.0 |
| 9.     | do            | B                | 830               | 79                                  | 55.4  | -1.3 | +12.7 | 14.3 | 83.2 |
| 10.    | do            | B                | 930               | 24                                  | 68.9  | -0.1 | +5.8  | 4.7  | 79.1 |
| 11.    | Bright anneal | Uncoated         |                   |                                     | 76.8  | 0.0  | +3.9  | 0    | 59.4 |
| 12.    | do            | A                | 630               | 64                                  | 66.3  | -0.1 | +9.7  | 12.0 | 60.0 |
| 13.    | do            | A                | 630               | 20                                  | 70.0  | -1.3 | +5.7  | 7.1  | 55.4 |
| 14.    | do            | A                | 630               | 61                                  | 66.9  | +1.6 | +10.3 | 11.9 | 58.5 |

The L term refers to the lightness of color and corresponds to the lightness scale used in the Munsell Color System. Low values of L are associated with dull surfaces while bright surfaces give numerically large L values. L indicates the quantity of black or white contained in the hue (color). Higher L values are closer to white and lower L values are closer to black. The "a" term requires a positive or negative prefix sign to indicate whether red or green hues are present. The positive prefix is for red hues and the negative prefix is for green hues. The size of the number indicates the strength or amount of the particular hue present in the total color. The "b" term is similar with the positive prefix indicating yellowness and the negative prefix indicating blueness. The size of the number indicates the strength or amount of yellow or blue present in the total color. The Δ E value is a calculated color difference that exists between the selected standard and the sample being examined. It is equal to the square root of  $(\Delta L)^2 + (\Delta a)^2 + (\Delta b)^2$ . Uncoated samples 1 and 11 were used as the selected standard. The haze value is a ratio of the intensity of diffused light to reflected light times 100. Standard rhodium mirrors have a haze value of 11.0 while sandblasted surfaces have haze values near 100.

A study of Table III reveals how a wide range of colors can be imparted to the coating by varying either the coating solution, curing temperature, material finish and/or coating thickness. The tests show L values ranging from 55.4 to 70.0, "a" values ranging from -1.5 to +1.6 and "b" values ranging from 4.5 to 17.7.

It will be apparent to those skilled in the art that the novel principles of the invention disclosed herein in connection with specific examples thereof, will suggest various other modifications and applications of the same. It is accordingly desired that in construing the breadth of the appended claims they shall not be limited to the specific examples of the invention disclosed herein.

I claim:

1. A method of providing a decorative exposed metallic surface with a transparent cured coating which protects against

marring, marking and staining, comprising the steps of: coating said metallic surface with an aqueous solution of magnesium, ammonium, chromate and phosphate ions, said aqueous solution having a molar concentration of said ions of between about 0.01 and 1.5 moles of said ions per 100 ml. of water, said ions being proportionately present in said aqueous solution as 0.01-28 mole percent magnesium ion, 5-22 mole percent ammonium ion, 4-26 mole percent chromate ion and 33-67 mole percent phosphate ion; and curing said coating at an elevated temperature so as to render it substantially water insoluble.

5 5. A method according to claim 1 wherein said ions are proportionately present in said aqueous solution as 16-26 mole percent magnesium ion, 7-15 mole percent ammonium ion, 7-21 mole percent chromate ion and 45-65 mole percent phosphate ion.

10 6. A method according to claim 1 wherein said molar concentration of said ions in said aqueous solution is between about 0.25 and 0.8 moles of said ions per 100 ml. of water.

15 7. A method according to claim 1 for providing a colored coating which includes the step of adding pigments or dyes to the aqueous coating solution.

8. A method according to claim 1 wherein said coating is cured by heating said metallic surface at a temperature of

40 45 from about 400° F. to about 1,900° F. for a period of from 2 seconds to about 4 hours.

9. A method according to claim 1 adapted to protect a

45 50 metallic surface selected from the group consisting of stainless

steel, brass, aluminum, silver, zinc, copper, plain carbon steel,

lead, chromium, nickel, gold, platinum, and alloys of said

metals.

10. A method according to claim 6 wherein said metallic sur-

face is stainless steel.

11. A composite article comprising a layer of metal having a

45 55 decorative exposed surface and at least one layer of a substan-

tially water insoluble, cured coating of magnesium cations and

anionic polymeric chains of chromium, oxygen, and

50 55 phosphorus atoms, adhered to said surface; said coating hav-

ing been formed from an aqueous solution of magnesium, am-

monium, chromate and phosphate ions having a molar con-

centration of between 0.01 and 1.5 moles of said ions per 100

ml. of water and having said ions proportionately present as

0.01-28 mole percent magnesium ion, 5-22 mole percent

50 55 ammonium ion, 4-26 mole percent chromate ion and 33-67

mole percent phosphate ion; said coating providing said

metallic surface with protection against marring, marking and

55 60 staining.

12. An article according to claim 8 wherein each layer of said

coating is less than about 0.0005 inches thick.

13. An article according to claim 8 wherein said metal is

selected from the group consisting of stainless steel, brass,

aluminum, silver, zinc, copper, plain carbon steel, lead, chro-

mium, nickel, gold, platinum and alloys of said metals.

11. An article according to claim 10 wherein said metal is stainless steel.

12. An article according to claim 8 wherein said water insoluble cured coating is transparent and substantially colorless.

13. An article according to claim 8 wherein said water insoluble cured coating is transparent and colored.

14. An article according to claim 8 wherein said metal is stainless steel and wherein each layer of said coating is less than about 0.0005 inches thick.

15. In the method of producing a stainless steel trim member, wherein a stainless steel strip is shaped into a trim member having an exposed surface and at least one contact surface, the improvement which comprises: coating said contact surface with an aqueous solution of magnesium, ammonium, chromate and phosphate ions, said aqueous solution having a molar concentration of said ions of between about 0.01 and 1.5 moles of said ions per 100 ml. of water, said ions being proportionately present in said aqueous solution as 0.01 - 28 mole percent magnesium ion, 5 - 22 mole percent ammonium ion, 4 - 26 mole percent chromate ion and 33 - 67 mole percent phosphate ion; and curing said coating at an elevated temperature so as to render it substantially water insoluble.

16. A method according to claim 15 including the steps of coating said exposure surface with said aqueous solution and curing said coating on said exposure surface.

17. A method according to claim 15 wherein said coating is cured by heating said metallic surface at a temperature of from about 400° F. to about 1,900° F. for a period of from about 2 seconds to about 4 hours.

18. A stainless steel trim member having an exposed surface, a contact surface and at least one layer of a substantially water insoluble cured coating of magnesium cations and anionic polymeric chains of chromium, oxygen and phosphorus atoms, adhered to said contact surface; said coating having been formed from an aqueous solution of magnesium, ammonium, chromate and phosphate ions having a molar concentration of between 0.01 and 1.5 moles of said ions per 100 ml. of water and having said ions proportionately present as 0.01 - 28 mole percent magnesium ion, 5 - 22 mole percent ammonium ion, 4 - 26 mole percent chromate ion and 33 - 67 mole percent phosphate ion.

19. A stainless steel trim member according to claim 18 wherein at least one layer of said coating is adhered to said exposure surface.

20. A stainless steel trim member according to claim 19 wherein each layer of said coating is less than about 0.0005 inches thick.

21. An assembly comprising a stainless steel trim member in combination with a metallic body member less noble in the electromotive series than stainless steel; said stainless steel trim member having an exposed surface, a contact surface abutting said metallic body member and at least one layer of a substantially water insoluble cured coating of magnesium cations and anionic polymeric chains of chromium, oxygen and phosphorus atoms, adhered to said contact surface; said coating having been formed from an aqueous solution of magnesium, ammonium, chromate and phosphate ions having a molar concentration of between 0.01 and 1.5 moles of said ions per 100 ml. water and having said ions proportionately present as 0.01 - 28 mole percent magnesium ion, 5 - 22 mole percent ammonium ion, 4 - 26 mole percent chromate ion and 33 - 67 mole percent phosphate ion.

22. An assembly according to claim 21 wherein at least one layer of said coating is adhered to said exposure surface.

23. An assembly according to claim 22 wherein each layer of said coating is less than about 0.0005 inches thick.

24. A method of providing an exposed metallic surface from the group consisting of stainless steel, brass, aluminum, silver, zinc, copper, plain carbon steel, lead, chromium, nickel, gold, platinum, and alloys of said metals with protection against marring, marking, staining, and corrosion, which comprises the steps of: coating said metallic surface with an aqueous solution of magnesium, ammonium, chromate and phosphate ions, said aqueous solution having a molar concentration of said ions of between about 0.01 and 1.5 moles of said ions per 100 ml. of water, said ions being proportionately present in said aqueous solution as 0.01 - 28 mole percent magnesium ion, 5 - 22 mole percent ammonium ion, 4 - 26 mole percent chromate ion and 33 - 67 mole percent phosphate ion; and curing said coating by heating said metallic surface at a temperature of from about 400° F. to about 1,900° F. for a period of from 2 seconds to about 4 hours, so as to render it substantially water insoluble.

\* \* \* \* \*